

## UNITED STATES PATENT OFFICE

CYRIL J. STAUD AND JAMES T. FUESS, OF ROCHESTER, NEW YORK, ASSIGNORS TO  
EASTMAN KODAK COMPANY, OF ROCHESTER, NEW YORK, A CORPORATION OF NEW  
YORK

## NITRATION OF CELLULOSE WITH A NITROGEN OXIDE

No Drawing.

Application filed December 31, 1930. Serial No. 505,965.

This invention relates to the nitration of cellulose with a higher oxide of nitrogen in either gaseous or liquid form.

An object of our invention is to provide a nitrating agent more economical than that ordinarily used, especially where a comparatively small amount of nitration is desired. Previously cellulose nitrate has been prepared by the action of a mixture of nitric and sulphuric acids upon cellulose. The present invention contemplates the use especially of  $\text{NO}_2$  which may be obtained from the gases used in the preparation of nitric acid. The use of oxide of nitrogen does away with the necessity of preparing the nitric acid from the oxide.

The following examples are given as illustrative of our invention with the use of the nitrogen oxide in the gaseous and in the liquid state.

*Example I*

About 10 grams of cellulose in the form of cotton linters may be fluffed so as to insure uniform treatment. With some forms of cellulose such as cotton dust this procedure is obviously entirely unnecessary and may even be omitted in the present process. The material is then placed in a vacuum desiccator and the air is removed therefrom. Gaseous  $\text{NO}_2$  is then introduced until a concentration of  $\text{NO}_2$  in the vessel is quite high. The cellulose is allowed to stand in this atmosphere until the desired nitration is obtained. If desired, the gas may be changed at intervals during this treatment or continuously passed through the cellulose. Nitration has been found to take place after 1-2 hours.

However, the treatment is preferably continued for 18 hours. The resulting product showed upon analysis a nitrogen content of about 1.38% nitrogen.

*Example II*

About 10 grams of cellulose (cotton linters preferred) are placed in about 100 c. c. of liquid  $\text{NO}_2$ , and kept at a temperature of 10° C. After allowing the material to re-

main at this temperature for the desired time, the mixture is removed and the  $\text{NO}_2$  may be driven off by pouring off the liquid and boiling the remaining  $\text{NO}_2$  or by blowing it out by air. If desired, the remaining material may be washed in a dilute solution of sodium bicarbonate. The amount of liquid  $\text{NO}_2$  used and the temperature and time may be varied if desired. It has been found that this reaction proceeds very rapidly at first, but then decreases perceptibly in rate so that with further treatment the nitrogen content increases very slowly. When time is a factor, therefore, a very short time may be used, but if the nitrogen content is the controlling factor the process may be allowed to run 72 hours or even longer, if desired. It was found upon carrying the process out for 48 hours that the nitrogen content of the resulting product was 11.30-11.95%. Other oxides of nitrogen such as  $\text{N}_2\text{O}_3$  and  $\text{N}_2\text{O}_5$  may be used instead of the dioxide or its dimer  $\text{N}_2\text{O}_4$  as the nitrating agent in the present process.

Any cellulosic material which is compatible with the process of this invention may be used instead of cotton linters. Suitable cellulosic materials that may be used are scrap cotton cloth, long fibered cotton, materials containing alpha, beta and gamma cellulose and high grade wood pulps or other like material.

As pointed out previously the time of treatment of the cellulose with the oxide of nitrogen may be varied within wide limits, depending on the nitrogen content desired. Although in the use of the liquid oxide of nitrogen as the nitrating agent a temperature below the boiling point of the oxide is desirable, in the treatment of the cellulose with the gaseous nitrating agent it is even desirable to warm the gases which pass into the reaction chamber. It is also desirable though not essential that enough gas is passed into the chamber so that the pressure therein be above atmospheric. Obviously various other technical details may be varied by the operator of this process without going outside the scope of this invention.

What we claim as our invention and desire

to secure by Letters Patent of the United is:

1. A process of nitrating cellulose which comprises treating the cellulose with a bath comprising a nitrating agent substantially consisting of a nitric oxide.

2. A process of nitrating cellulose which comprises treating the cellulose with a higher oxide of nitrogen in gaseous form.

3. A process of nitrating cellulose which 10 comprises treating the cellulose with a bath comprising a nitrating agent substantially consisting of a higher oxide of nitrogen in liquid form.

15

80

20

85

25

90

30

95

35

100

40

105

45

110

50

115

55

120

60

125

65

130

4. A process of nitrating cellulose which comprises treating the cellulose with gaseous  $\text{NO}_2$ .

5. A process of nitrating cellulose which comprises treating the cellulose with a bath comprising a nitrating agent substantially consisting of liquid  $\text{NO}_2$ .

Signed at Rochester, New York, this 29th day of December 1930.

CYRIL J. STAUD.  
JAMES T. FUESS.

75  
100